

## UNITED STATES PATENT OFFICE

2,109,792

## METHOD OF TREATING PECTIN

Gordon Manley Cole and Raymond Edward Cox,  
Corona, Calif., assignors to California Fruit  
Growers Exchange, Los Angeles, Calif., a cor-  
poration of California

No Drawing. Application February 18, 1935,  
Serial No. 7,075

9 Claims. (Cl. 99—132)

This invention relates to a method of treating pectin sols whereby certain fundamental and inherent characteristics of the pectin may be changed.

5 Pectin is used commercially in the manufacture and production of various products, important among which are jams, and jellies. Each trade requires that the pectin have certain characteristics, although these characteristics may 10 differ for different trades and uses; that is to say, certain users require pectin with a uniformly slow setting rate, whereas, a pectin with a fast setting rate is required by others. Heretofore, it has been difficult, if not impossible, for the pectin 15 manufacturer to manufacture pectin with a predetermined and uniform setting time or rate. Different source material and extraction methods produce pectins with differing and generally uncontrollable setting characteristics. There is, 20 therefore a distinct need for some method whereby the setting time or setting rate of pectin can be controlled or modified.

This invention is based upon the discovery that it is possible to alter, at will, one of the inherent, 25 intrinsic and fundamental characteristics of pectin, namely, its setting time, or its inherent ability to cause gelation to proceed in a jelly batch at a certain definite rate. By the method and means of this invention, the setting time of any 30 previously extracted pectin may be changed in the desired direction.

The setting time as used in this specification and in the appended claims means that interval of time which elapses between the instant all 35 the ingredients of the jelly batch, consisting of standard proportions of sugar, pectin, acid, and total solids, are placed in the final container, after cooking, and that instant at which gelation of the whole into a coherent mass may be observed.

Generally stated, the method comprises contacting the pectin with a reagent adapted to alter materially the intrinsic setting time of said 45 previously extracted pectin, and maintaining the reagent in contact with the pectin for a time and at a temperature insufficient to destroy the gelation characteristics of the pectin or materially affect the texture of the gel which may subsequently be formed from such treated pectin.

50 The treating reagent, before being brought into contact with the pectin sol, may be either liquid or gaseous, aqueous or anhydrous. The preferred reagent is an acid, an acidic, or an acid-forming substance. For convenience in handling and application of the reagent, a liquid may be used as a carrier. The reagent so added should preferably not react with the sol in any way so as to precipitate the pectin contained therein 55 during the period of time in which the retarda-

tion of the pectin is proceeding. An organic acid illustrates a desirable treating agent.

Accordingly, an object of this invention is to disclose and provide methods and means of changing or altering the setting time of pectins 5 in sol form.

Another object of this invention is to disclose and provide methods and means whereby it is possible to alter the setting time characteristics of pectins in sol form to any desired and definite, 10 predetermined time.

A further object of this invention is to disclose and provide methods and means of treating pectin sols of various degrees of purity for the purpose of changing the inherent setting time 15 characteristics, and in particular to retard the setting rate or lengthen the setting time.

Another object of this invention is to disclose and provide methods and means of treating pectin sols with an acidic reagent whereby the setting time may be retarded or speeded up to any 20 desired and predetermined time.

The objects and advantages of this invention will be apparent from a description of a preferred process and product embodied in the invention 25 and will present themselves to those skilled in the art in the contemplation and use of the invention.

It is to be understood that this invention is directed to the treatment of pectin in sol form, and particularly to the treatment of a pectin 30 which has been previously extracted from a cellulose source material. Various methods of extraction are known and need not be described herein. In such previously known methods, the pectin is precipitated from the extracts with alcohol, by salting out, or by the so-called aluminum precipitation process disclosed in Patent No. 1,497,884.

It has been determined that the process of this invention is applicable to pectins extracted from 40 any source, such as, for example, citrus peel, apple pomace, etc. Moreover, the process does not appear to be influenced by the method of extraction, precipitation, or purification used prior to the application of the process of this invention. 45 The sol, being treated in accordance with this invention, may be either of a technical quality or of a more extensively purified quality.

In the following descriptions the process is illustrated as applied to the treatment, in sol form, 50 of commercial pectins having a setting time of about 9 seconds, and to the treatment of pectin in sol form obtained from the HCl extraction of citrus pulp at a pH of about 1.6. We desire it to be understood that the treatments described are 55 given as illustrations of the invention and the invention is not to be limited to the examples given, but the treatment may be modified in various manners depending upon how the pectin sols are formed, whether by original extraction 60

of the pectin from raw materials, or by redispersing pectin which has previously been precipitated from extraction liquors. The pectin to be treated may be purified by known means.

- 5 Again, we desire it to be understood that this invention relates to and is applicable to pectin in sol form extracted from any source, such as, for example, apple pomace, citrus peel, etc. Furthermore, this process does not seem to be influenced by the method of extraction, or purification of the pectin, that is, whether it be a relatively pure sol made by dispersing a highly purified pectin, or a sol containing appreciable amounts of extraction impurities.
- 15 As has been stated hereinbefore, the method of the invention contemplates acting upon a pectin sol with a treating agent, so as to alter the inherent time of set of the pectin therein contained. The preferred process is carried out 20 by adding a suitable acid to the pectin sol, and in order to illustrate the process and the results to be obtained thereby, the following examples are given.

25 62.5 grams of a 160 grade commercial powdered pectin having a setting time of about 9 seconds were dispersed in 5 kg. of 1.16 normal HCl, yielding a 1 1/4% pectin sol having a pH of approximately 0.1, as measured by using a quinhydrone electrode in conjunction with a standard 30 calomel half-cell, standardized against a standard buffer solution. 400 cc. portions of this sol were taken from the main supply at intervals shown in Table I, the main supply being held at room temperature throughout the experiment.

35 The treatment of the pectin sol, after removal from the main supply, consisted of precipitation of the pectin from the sol with an equal volume of 95% alcohol, straining the pectin therefrom, adding it to 400 cc. of 50% alcohol, straining and 40 repeating the rinse twice more. The resulting pectin was air dried, thence ground to 65 mesh and standard jellies of satisfactory texture were made.

45 A "standard jelly" as herein used is composed of approximately 65% sugar solids, plus 2 cc. of standard preservers acid (1/2 pound crystalline tartaric acid to 1 pint of distilled water) per 170 ml. volume of finished jelly, and sufficient pectin to set the whole into a jelly of suitable texture 50 and resiliency.

55 Comparative jelly grades of various pectins are usually calculated on an ash and moisture free basis. The comparison of the various jelly grades is thereby on an equal basis, namely, a basis wherein the entire pectin is considered as though pure pectin, entirely free from ash and moisture.

TABLE I

60 1 1/4% pectin sol acidified with HCl to a pH of approximately 0.1 stored at room temperature

| Treating time                                 | Time of set | Jelly grade |
|-----------------------------------------------|-------------|-------------|
| (After treatment ash and moisture free basis) |             |             |
| 1 hour                                        | 9 sec.      | 180         |
| 4 hours                                       | 32 sec.     | 179         |
| 21 hours                                      | 95 sec.     | 178         |
| 45 hours                                      | 11 min.     | 202         |
| 2 days                                        | 28 min.     | 217         |
| 3 days                                        | 28 min.     | 226         |
| 5 days                                        | 23 min.     | 265         |
| 9 days                                        | (5)* min.   | 211±5       |

75 \*Jelly had set when examined after 5 minutes.

As can be seen by referring to Table I, the pectin obtained from the pectin sols, treated as hereinbefore stated, had its intrinsic setting time greatly changed. The sample treated for 4 hours shows an appreciable retardation in setting time and from then on until the third day, whereupon the setting time begins to speed up and so continues up until the ninth day where the experiment was ended. A further interesting and entirely unexpected phenomenon has been discovered in that the jelly grade, or ability to produce jellification, in a standard jelly, has greatly increased along with retardation, for, as will be noted from Table I, the jelly grade values (on an ash and moisture-free basis), increase from 15 approximately 180 to as high as 265.

10 By the term jelly grade of a pectin is meant the ability of a pectin to form a satisfactory jelly under standardized conditions.

15 Pectin as supplied commercially is standardized 20 as to its jellifying strength. For example, a pectin which is capable of setting into a jelly of standard strength and resiliency one hundred and sixty times its weight of sugar in standard 25 jelly containing 65% soluble solids, by weight, may be referred to as 160 grade pectin. The variations in grade of commercial pectin may be very wide.

20 This pectin is handled in commerce on a certain price per unit of jelly grade for a unit 30 weight, that is, 200 grade pectin should sell for double the price of the same weight of 100 grade pectin.

25 Attention is again called to the fact that after the pectin in a pectin sol has been retarded, by 30 further treatment with the acidic reagent, it may again be speeded up. This is well demonstrated by the samples treated for 5 days and 9 days respectively. The 5 day treatment yielding a pectin setting in 23 minutes, and the 9 day 40 treatment a pectin setting in less than 5 minutes.

30 Although the foregoing example showed treatment of a pectin sol with acid at room temperature, it has been found that by increasing the temperature of the acidic pectin sol we will 45 hasten the desired results by cutting down the length of treating time. However, there is a maximum limit above which the temperature should, preferably, not go, namely about 85° C. A preferred temperature would be in the range of 50 40°-60° C.

35 Likewise it has been found that the more drastic the treatment, the shorter will be the time necessary for such a treatment. More specifically, a pectin sol treated with an acid at a pH of 0.1 will take a much shorter treating time than a sol treated at a pH of 1.8. The above figures are not meant to be maximum and minimum limits for the pH, however, since pH is a factor which is variable and may be adjusted to suit the 60 plant operations, or so adjusted that the maximum setting time retardation will be accomplished in the shortest possible time and at the least expense, and with the greatest gain in jelly grade. The use of too high a concentration of 65 acid, however, should be avoided, as some degradation of the pectin might take place, along with loss of jelly strength. Nevertheless, the use of too low a concentration of acid denoted by a pH of approximately 2.5 entails continuing the 70 storage time for an extremely long period, far beyond any economic or practical limit.

75 Notwithstanding that the examples given have dealt with purified pectins dispersed in acid solutions, we want to make it clear that pectin sols 75

direct from the extraction may have the setting characteristics of the pectin changed by increasing the temperature of the extracted pectin sol and letting it stand in the presence of the extraction or added acid. Such an example appears hereinafter.

A pectin sol obtained from the extraction of citrus pulp with HCl at a pH of approximately 1.6 was stored at a temperature of 40°-50° C. for 1.6 was stored at a temperature of 40°-50° C. for 10 164 hours. The concentration of pectin in this sol was about 1%. As is shown in Table II, the time of set was retarded from 48 seconds to 455 seconds, over a period of 148 hours. It is also apparent that the jelly grade increased from 178 15 to 185. Although Table II does not show definitely the effects of continued storage longer than 164 hours, yet it does indicate that the setting time is speeding up and the jelly grade decreasing.

TABLE II

| Storage time in hours | Setting time in seconds | Jelly grade |
|-----------------------|-------------------------|-------------|
| 25                    | Seconds                 |             |
| 0                     | 48                      | 178         |
| 54                    | 66                      | 175         |
| 77                    | 190                     | 180         |
| 103                   | 275                     | 180         |
| 124                   | 285                     | 185         |
| 148                   | 455                     | 185         |
| 30                    | 390                     | 160         |

At a higher pH, namely, 1.6, the set retardation proceeds more slowly for a given time and temperature than it would at a lower pH in the order of 0.5.

The reagent mentioned hereinbefore has been hydrochloric acid; however, other inorganic acids such as phosphoric acids, nitric, and sulfuric acid will also apply as will organic acids, citric, lactic, 40 etc. Results similar to those obtained by HCl may be obtained by using chlorine gas, hydrogen chloride, hydrogen sulfide, sulfur trioxide or sulfur dioxide, etc., will also act to retard the set of pectin in sol form.

We have found that a 1 to 1½% pectin sol is the most suitable concentration to deal with, but our process of treating pectin is applicable to concentrations greater than 0% and less than 5%. The upper limit of 5% is mentioned as that 50 limit beyond which production costs and trouble in handling, due to the great viscosity of the sols, would be too great for the process to be economically feasible.

It is therefore evident, from the descriptions given hereinabove, that a process has been disclosed which permits the manufacturer, or user, or dealer to alter at will the setting time of pectin in sol form.

Although we have stated as a primary object 60 of this disclosure, the change of setting time, still we have made it apparent that there are other advantages, for example, the improvement of jelly grade of the pectin sol. Furthermore, pectin precipitated from pectin sols so treated, at optimum conditions of time, pH, concentration, and temperature, will have a lower ash content and will be lighter in color.

Although specific materials have been mentioned as suitable reagents for the process of this 70 invention, they have been set forth for the purpose of illustration only, and the invention is not limited thereto. Any and all changes, modifications, or alterations coming within the scope of the appended claims are to be considered em-

We claim:

1. A method of treating pectin which comprises contacting pectin in sol form, after substantial separation of the pectin from its source material, with an acidic reagent adapted to materially alter the intrinsic setting time of the pectin, the pectin being maintained in contact with the reagent for a period of time and at a temperature insufficient to destroy the gelation characteristics of the pectin but sufficient to materially alter the intrinsic setting time thereof. 5

2. A method as defined in claim 1 in which the reagent comprises an acid.

3. A method of treating pectin as defined in claim 1 in which the reagent is an acidic gas 15 from the group consisting of hydrogen chloride, chlorine, hydrogen sulfide, sulfur dioxide and sulfur trioxide.

4. A method of treating pectin as defined in claim 1 in which the reagent is maintained in 20 substantial contact with the pectin for a period of time from about 1 to about 148 hours.

5. A method of treating pectin whereby the setting time thereof is altered, comprising contacting the pectin in sol form, after substantial 25 separation of the pectin from its source material, with an acidic reagent, and maintaining such contact for a time and at a temperature sufficient to materially alter the setting time of the pectin, then separating the pectin from the solution and washing the pectin to diminish residual 30 acidity thereof.

6. A method of increasing the setting time of pectin, comprising contacting the pectin in sol form, after substantial separation of the pectin 35 from its source material with an acidic reagent at a pH below 2.5, and for a time and at a temperature sufficient to materially increase the setting time of the pectin.

7. A method of converting a previously separated, relatively quick-setting pectin into a relatively slow-setting pectin, which comprises dissolving the pectin to form a pectin sol, subjecting the pectin sol to treatment with an acidic reagent adapted to materially increase the setting 40 time of the pectin, maintaining said treatment for a time and at a temperature insufficient to destroy the gelation characteristics of the pectin but sufficient to materially increase the setting time thereof, and then reducing the 50 pectin to dry form, thereby recovering a relatively slow-setting pectin. 45

8. A method of converting a previously separated, relatively quick-setting pectin into a relatively slow-setting pectin, which comprises dissolving the pectin to form a pectin sol, subjecting the pectin sol to treatment with an acidic reagent adapted to materially increase the setting 55 time of the pectin, maintaining said treatment for a time and at a temperature insufficient to destroy the gelation characteristics of the pectin but sufficient to materially increase the setting time thereof.

9. A method of treating pectin which comprises substantially separating pectin from its 65 source material, contacting the pectin in sol form with an acidic reagent adapted to materially alter the intrinsic setting time of the pectin, the pectin being maintained in contact with the reagent for a period of time and at a temperature insufficient to destroy the gelation characteristics of the pectin but sufficient to materially alter the intrinsic setting time thereof. 70

GORDON MANLEY COLE.